

July 14, 1931.

W. O. STODDARD, JR

1,814,643

COMPOSITE MATERIAL

Filed April 9, 1925



Fig. 1



Fig. 2

INVENTOR

William O. Stoddard, Jr.

BY

John Barnes

ATTORNEY

## UNITED STATES PATENT OFFICE

WILLIAM O. STODDARD, JR., OF DETROIT, MICHIGAN

## COMPOSITE MATERIAL

Application filed April 9, 1925. Serial No. 21,976.

It is the primary object of my invention to provide a composite material in the nature of a fabric adapted for use as artificial leather or like products.

Among the various other objects of my invention are the use of unspun and unwoven materials, making possible the use of low-priced materials with a consequent economy in the finished product.

While my invention is adapted for many uses and may be fabricated in a number of different ways, it is particularly adapted for use as artificial leather and is preferably made by the super-posing of layers of material beginning first with a layer such as cotton, on which is disposed a layer such as jute, flax, hair or other fibre, then disposing another layer of cotton over the mass, followed by another layer of jute, flax, hair or other fibre, the two layers of fibrous material being so disposed that the lines of the fibres of the two different layers will intersect. This intersection of fibres lends material strength to the composition.

With the above objects and advantages in view, my invention consists in the arrangement, combination and construction of the various parts of my improved composition, as well as the method of making the same, as described in the specification, claimed in my claims and shown in the accompanying drawings, in which:

Fig. 1 is a top or plan view of my improved material with parts broken away to show its construction.

Fig. 2 is a sectional view showing the same.

I have shown a section of composite material composed of a layer of cotton 5, upon which is placed a layer of jute, flax, hair or other fibre 6, with the strands thereof curled, twisted or otherwise distorted in a manner most easily or usually obtained according to the particular material used. Upon the layer 6 is super-posed another layer 7 of cotton 45 and upon this is placed another layer 8 of fibrous material so disposed that at least some of the strands of the fibre will cross with those in the layer 6. Upon the layer 8 is disposed another layer 9 of cotton. All of 50 the layers are glued or cemented together

with rubber or other cement, so as to make a unitary mass and a covering 10 for the top of the material is provided, consisting of rubber, pyroxyline or linseed oil compositions, or any other well-known combination 55 of materials such as are usually employed in the provision of artificial leather coatings.

The super-posing, or laminating, of the layers of material with the fibres of the fibrous layers intersecting each other provides 60 a strong composition and makes unnecessary the weaving or spinning of the materials. Likewise the use of the fibrous material without necessity of the fibres of each layer being stranded, or otherwise worked 65 (making use of them as they may be found) cheapens the finished product, as does the fact that the grade of material used need not be high. The cotton layers, in particular, 70 need not be of high-grade material, inasmuch as the cotton lends little or no strength to the mass, but acts as a filler to give bulk to the composition.

It will be understood, of course, that as many layers of cotton or other fillers, and as 75 many layers of jute or other fibrous materials, may be utilized as is desired by the maker to suit the particular need for which the material is to be used.

It will be obvious that various changes 80 may be made in the arrangement, combination and construction of the various elements of my invention and in the method utilized in making the same, without departing from the spirit of my invention, and it is my intention 85 to cover by my claims such changes as may be reasonably included within the scope thereof.

What I claim is:

1. As an article of manufacture a substitute 90 for woven covering materials which consists of a pliable mass composed of a plurality of superposed relatively thin layers of unspun and unwoven fibers, having the intervening layers composed of fibers of relatively 95 greater tensile strength than the fibers of the alternate layers, the fibers of each of said intervening layers being disposed in nonparallel and entangling relation to each other and in nonparallel relation to the fibers of 100

the other intervening layers, said layers being adhesively secured to each other, and a non-fibrous waterproof cover adhesively secured on one side of said mass.

2. As an article of manufacture a substitute for woven covering material which consists of a pliable mass composed of a plurality of laminated layers of unspun and unwoven fibers having the intervening layers composed of interlocking fibers of relatively

10 greater strength than the fibers of the alternate layers, said layers being adhesively secured to each other, and a non-fibrous substantially waterproof substance adhesively secured to one side of said mass.

15 3. As an article of manufacture a substitute for woven covering material which consists of a pliable mass composed of a plurality of layers of unspun and unwoven fibers, having the alternate layers composed of flocculated cotton fibers, and the intervening layers composed of entangled fibers of relatively greater strength than the cotton fibers, said layers being cemented together, and a substantially waterproof cover adhesively secured to one side of the mass.

4. As an article of manufacture, a substitute for woven covering material which consists of a pliable mass composed of a plurality of laminated layers of unspun and unwoven fibers having some of the layers composed of interlocking fibers of relatively greater strength than the fibers of other of said layers, said layers being adhesively secured to each other and a substantially waterproof cover adhesively secured to the mass.

WILLIAM O. STODDARD, JR.